# EUROPEAN PATENT SPECIFICATION

(11) **EP 0 345 483 B1**
(45) Date of publication and mention of the grant of the patent: **28.12.1994**
(21) Application number: 89108559.9
(22) Date of filing: 12.05.1989
(51) Int. Cl.: G03C 1/035, G03C 1/12, G03C 5/16, G03C 1/825

(54) **Light-sensitive elements for radiographic use and process for the formation of an X-ray image**
Lichtempfindliche Elemente zur radiographischen Verwendung und Verfahren zur Herstellung eines X-Strahlungsbildes
Eléments sensibles à la lumière pour usage radiographique et procédé de formation d'une image de rayons X

(30) Priority: 09.06.1988 IT 2090388
(43) Date of publication of application: 13.12.1989
(73) Proprietor: MINNESOTA MINING AND MANUFACTURING COMPANY, St. Paul, Minnesota 55133-3427 (US)
(72) Inventor: Cavallo, Elio, I-17016 Ferrania/Savona (IT); Bussi, Giuseppe, I-17016 Ferrania/Savona (IT)
(74) Representative: Allaix, Roberto

(56) References cited:
- US-A- 4 574 115
- US-A- 4 639 411
- PATENT ABSTRACTS OF JAPAN vol. 11, no. 308 (P-624)(2755) 08 October 1987,& JP-A-62 099748
- PATENT ABSTRACTS OF JAPAN vol. 11, no. 151 (P-576)(2598) 16 May 1987,& JP-A-61 285445
- PATENT ABSTRACTS OF JAPAN vol. 13, no. 291 (P-893)(3639) 06 July 1989,& JP-A-01 073336

## Description

### FIELD OF THE INVENTION

The present invention refers to light-sensitive silver halide elements to be used in radiography and, more in particular, to light-sensitive silver halide elements to be used with intensifying screens to obtain improved X-ray images.

### BACKGROUND OF THE INVENTION

In radiography, and particularly in medical radiography, light-sensitive elements having silver halide emulsion layers coated on one side of a transparent base are used. It is known to be more preferable to use silver halide emulsions on both sides to obtain better developability as compared to single-side coated elements. Light-sensitive elements having silver halide emulsion layers coated on one side and, more preferably, on both sides of the base are generally used in association with intensifying screens in order to reduce the X-ray exposure necessary to obtain the required image. Generally, one intensifying screen is used on each side of the light-sensitive element. The silver halides used in the light-sensitive elements are sensitive or sensitized to a region of the electromagnetic spectrum corresponding to the wavelength of the light emitted by the luminescent materials used in the intensifying screens, thus obtaining significant amplification factors.

The quality of image obtained upon exposure and development of said radiographic elements is negatively affected by light scattering and crossover exposure.

Light scattering occurs both in single and double emulsion layer coated radiographic materials when light emitted by one screen is diffused (scattered) by silver halide grains causing a reduction in image sharpness.

Crossover exposure, which also causes a reduction in image sharpness, occurs in double emulsion layer coated radiographic materials when light emitted by one screen passes through the adjacent emulsion layer and the support and, the light having been spread by the support, image-wise exposes the emulsion layer on the opposite side of the support.

The crossover exposure causes poor definition even if light-sensitive elements are used which employ reduced silver halide coverages to lower the costs or increase the processing speed of the element. In fact, the decrease of the emulsion turbidity increases the amount of light available for crossover and therefore worsens the image.

To reduce the crossover phenomenon, dyes or pigments can be used within the photographic element. The absorption of said dyes or pigments is in a region of the electromagnetic spectrum corresponding to the wavelength of the light emitted by the intensifying screens. The dyes or pigments absorb some of the light emitted by the intensifying screen so that imaging of the rear emulsion by the forward screen is reduced by absorbance of the light from the forward screen by the anticrossover layer. These dyes or pigments are eliminated during the photographic developing, fixing and washing process of the exposed material; they can be for instance washed away or, more preferably, bleached while processing the radiographic element.

The dyes can be incorporated in any layer of the light-sensitive element: in the emulsion layer, in an intermediate layer between the emulsion and the base, or in the subbing layer of the support base. It is preferred to incorporate the dyes in a layer different from that containing the emulsion to avoid possible desensitization phenomena. Since 1978, Minnesota Mining and Manufacturing Company has sold a radiographic element under the name of 3M Trimax™ Type XUD X-Ray Film to be used in combination with 3M Trimax™ Intensifying Screens. Such radiographic element comprises a transparent polyester base, each surface of which has a silver halide emulsion layer sensitized to the light emitted by the screens. Between the emulsion and the base is a gelatin layer containing water-soluble acid dyes, which dyes can be decolorized during processing and have an absorption in a region of the electromagnetic spectrum corresponding to the wavelength of the light emitted by the screens and of the spectral sensitivity of the emulsion. The dyes are anchored in the layer by means of a basic mordant consisting of polyvinylpyridine.

In the practical solution of reducing the crossover exposure by using a mordanted dye layer (as described for instance in the European Patent Application 101,295), some problems are created which up to now have not yet been solved properly. In fact, the improvement of image definition involves not only a natural decrease of the light-sensitive element sensitivity caused by the absorption of the transmitted and diffused light which otherwise would take part in the formation of a part of the image, but also the possibility of desensitization phenomena due to the migration of dye not firmly mordanted in the silver halide emulsion layer. There is also a problem with residual stain even after processing, the retention of significant quantities of thiosulfate from the fixing bath which causes image yellowing upon longtime storage on shelf, and lengthening of the drying times after processing because of element thickening.

Other approaches have been suggested to reduce crossover, as reported hereinbelow.

US Patent 3,923,515 discloses a relatively lower speed silver halide emulsion between the support and a higher speed silver halide emulsion layer to reduce crossover.

US Patent 4,639,411 discloses a photographic element, to be used with blue emitting intensifying screens,having reduced crossover, said element comprising coated on both sides of a transparent support a blue sensitive silver halide emulsion layer and, interposed between the support and and the emulsion layer, a blue absorbing layer comprising bright yellow silver iodide grains of a specific crystal structure.

Japanese Patent Application 62-52546 discloses a radiographic element of improved image quality comprising coated on both sides of a transparent support a light sensitive silver halide emulsion layer and, interposed between the support and the emulsion layer, a layer containing water insoluble metal salt particles having adsorbed on their surface a dye. Said dye has a maximum absorption within the range of ± 20 nm of the maximum absorption of said silver halide and corresponds to the light emitted by intensifying screens. Silver halides are disclosed as preferred metal salt particles.

US patent 4,751,174 (JP-A-62-99748) discloses a photosensitive material of improved image quality comprising, coated between a support and a light-sensitive silver halide emulsion layer, a silver halide emulsion layer having substantially no light-sensitivity, such as silver halide particles having a high fixing speed, finely divided silver halide particles, tabular silver halide particles, or particles with a sensitizing dye adsorbed thereon.

The approaches of using light-insensitive silver halide layers as anticrossover layers interposed between the support and the light-sensitive silver halide emulsion layers, although preferred to using dyes or pigments, encounter some problems such as the increase of silver coverage and bad bleaching characteristics in photographic processing (residual stain).

### SUMMARY OF THE INVENTION

In one aspect this invention is directed to substantially light-insensitive very fine grain low iodide silver bromoiodide grains, having adsorbed on their surface spectral sensitizing dyes to form a sharp absorption band (J-band).

In another aspect this invention is directed to a silver halide X-ray element to be used with X-ray intensifying screens comprising a transparent support base having coated on at least one of its sides a spectrally sensitized silver halide emulsion layer and, between the support base and the silver halide emulsion layer, a hydrophilic colloid layer containing substantially light-insensitive silver halide grains on which a spectral sensitizing dye is adsorbed, said dye adsorbed on said grains having absorption in a region of the electromagnetic spectrum corresponding substantially to the spectral sensitivity of the silver halide emulsion, wherein said substantially light-insensitive silver halide grains are low iodide silver bromoiodide grains having an average grain size in the range of from 0.01 to 0.1 µm adsorbed with said spectral sensitizing dye to form a J-band.

Said X-ray element offers advantages in crossover reduction without causing negative effects, such as significant loss of sensitivity, residual stain, image instability upon storage and excessive element thickening.

### DETAILED DESCRIPTION OF THE INVENTION

Accordingly, in one aspect, the present invention relates to a substantially light-insensitive silver halide emulsion comprising silver halide grains on which a spectral sensitizing dye is adsorbed, characterized by the fact that said silver halide grains are low iodide silver bromoiodide grains having an average grain size of from 0.01 to 0.1 µm adsorbed with said spectral sensitizing dye to form a J-band.

The term "low iodide grains" in the present invention means a total percentage of halide in the grains of more than 0.2 mole percent and less than 10 mole percent iodide. Preferably the silver iodide provided by the silver bromoiodide grains is limited to less than 5 mole percent of the total silver halide present in the grains, and more preferably less than 3 mole percent. Silver iodide grains of at least 1 mole percent are preferred to produce the desired J-band.

Said silver bromoiodide grains are substantially light-insensitive, that is they do not form any image upon conventional exposure (e.g. for a 10⁻² sec time) to radiations of a wavelength in the range from 420 to 700 nanometers and development in standard black and white and color developers. Such sensitivity can be generally described as being of less than 1 ASA. In the case of the emulsions of the present invention, they preferably are of a sensitivity lower than 10⁻¹ ASA. The grain size of said light-insensitive silver bromoiodide grains is particularly restricted. The grains are 0.1 µm or less in mean diameter. The minimum mean diameters of the grains are limited only by synthetic convenience. Typically, grains of at least 0.01 µm in mean diameter are employed. The light-insensitive silver bromoiodide grains of the present invention have adsorbed on their surface spectral sensitizing dyes that exhibit absorption maxima in the blue and/or green and/or red portions of the visible spectrum. Spectral sensitizing dyes according to this invention produce J aggregates if adsorbed on the surface of the silver halide grains and a sharp absorption band (J-band) with a bathocroinic shifting with respect to the absorption maximum of the free dye in aqueous solution. Spectral sensitizing dyes producing J aggregates are well known in the art, as illustrated by F. M. Hamer, Cyanine Dyes and Related Compounds, John Wiley and Sons, 1964, Chapter XVII and by T. H. James, The Theory of the Photographic Process, 4th edition, Macmillan, 1977, Chapter 8.

In a preferred form, J-band exhibiting dyes are cyanine dyes. Such dyes comprise two basic heterocyclic nuclei joined by a linkage of methine groups. The heterocyclic nuclei preferably include fused benzene rings to enhance J aggregation. The heterocyclic nuclei are preferably quinolinium, benzoxazolium, benzothiazolium, benzoselenazolium, benzimidazolium, naphthoxazolium, naphthothiazolium and naphthoselenazolium quaternary salts. J-band type dyes preferably used in the present invention have the following general formula (I):
wherein Z₁ and Z₂ may be the same or different and each represents the elements necessary to complete a cyclic nucleus derived from basic heterocyclic nitrogen compounds such as oxazoline, oxazole, benzoxazole, the naphthoxazoles (e.g., naphth{2,1-d}oxazole, naphth{2,3-d}oxazole, and naphth{1,2-d}oxazole), thiazoline, thiazole, benzothiazole, the naphthothiazoles (e.g., naphtho{2,1-d}thiazole), the thiazoloquinolines (e.g., thiazolo{4,5-b}quinoline), selenazoline, selenazole, benzoselenazole, the naphthoselenazoles (e.g., naphtho{1,2-d}selenazole, 3H-indole (e.g., 3,3-dimethyl-3H-indole), the benzindoles (e.g., 1,1-dimethylbenzindole), imidazoline, imidazole, benzimidazole, the naphthimidazoles (e.g., naphth{2,3-d}imidazole), pyridine, and quinoline, which nuclei may be substituetd on the ring by one or more of a wide variety of substituents such as hydroxy, the halogens (e.g., fluoro, bromo, chloro, and iodo), alkyl groups or substituted alkyl groups (e.g., methyl, ethyl, propyl, isopropyl, butyl, octyl, dodecyl, 2-hydroxyethyl, 3-sulfopropyl, carboxymethyl, 2-cyanoethyl, and trifluoromethyl), aryl groups or substituted aryl groups (e.g., phenyl, 1-naphthyl, 2-naphthyl, 4-sulfophenyl, 3-carboxyphenyl, and 4-biphenyl), aralkyl groups (e.g., benzyl and phenethyl), alkoxy groups (e.g., methoxy, ethoxy, and isopropoxy), aryloxy groups (e.g., phenoxy and 1-naphthoxy), alkylthio groups (e.g., ethylthio and methyithio), arylthio groups (e.g., phenylthio, p-tolythio, and 2-naphthylthio), methylenedioxy, cyano, 2-thienyl, styryl, amino or substituted amino groups (e.g., anilino, dimethylanilino, diethylanilino, and morpholino), acyl groups (e.g., acetyl and benzoyl), and sulfo groups,
R₁ and R₂ can be the same or different and represent alkyl groups, aryl groups, alkenyl groups, or aralkyl groups, with or without substituents, (e.g., carboxymethyl, 2-hydroxyethyl, 3-sulfopropyl, 3-sulfobutyl, 4-sulfobutyl, 2-methoxyethyl, 2-sulfatoethyl, 3-thiosulfatoethyl, 2-phosphonoethyl, chlorophenyl, and bromophenyl),
R₃ represents a hydrogen atom,
R₄ and R₅ can be the same or different and represent a hydrogen atom or a lower alkyl group of from 1 to 4 carbon atoms,
p and q are 0 or 1, except that both p and q preferably are not 1,
m is 0 or 1 except that when m is 1 both p and q are 0 and at least one of Z₁ and Z₂ represents imidazoline, oxazoline, thiazoline, or selenazoline,
A is an anionic group, B is a cationic group, and k and l may be 0 or 1, depending on whether ionic substituents are present. Variants are, of course, possible in which R₁ and R₃, R₂ and R₅, or R₁ and R₂ together represent the atoms necessary to complete an alkylene bridge.

More preferably said dye adsorbed on said substantially light-insensitive silver bromoiodide grains is represented by the following general formula (II):
wherein
R₁₀ represents a hydrogen atom or a lower alkyl group of from 1 to 4 carbon atoms (e.g. methyl, and ethyl),
R₆, R₇, R₈ and R₉ each represents a hydrogen atom, a halogen atom (e.g. chloro, bromo, iodo, and fluoro), a hydroxy group, an alkoxy group (e.g. methoxy and ethoxy), an amino group (e.g. amino, methylamino, and dimethylamino), an acylamino group (e.g. acetamido and propionamido), an acyloxy group (e.g. acetoxy group), an alkoxycarbonyl group (e.g. methoxycarbonyl, ethoxycarbonyl, and butoxycarbonyl), an alkyl group (e.g. methyl, ethyl, and isopropyl), an alkoxycarbonylamino group (e.g. ethoxycarbonylamino) or an aryl group (e.g. phenyl and tolyl), or, together, R₆ and R₇ and, respectively, R₈ and R₉ can be the atoms necessary to complete a benzene ring (so that the heterocyclic nucleus results to be, for example, an α-naphthoxazole nucleus, a β-naphthoxazole or a β,β′-naphthoxazole),
R₁₁ and R₁₂ each represents an alkyl group (e.g. methyl, propyl, and butyl), a hydroxyalkyl group (e.g. 2-hydroxyethyl, 3-hydroxypropyl, and 4-hydroxybutyl), an acetoxyalkyl group (e.g. 2-acetoxyethyl and 4-acetoxybutyl), an alkoxyalkyl group (e.g. 2-methoxyethyl and 3-methoxypropyl), a carboxyl group containing alkyl group (e.g. carboxymethyl, 2-carboxyethyl, 4-carboxybutyl, and 2-(2-carboxyethoxy)-ethyl), a sulfo group containing alkyl group (e.g. 2-sulfoethyl, 3-sulfopropyl, 4-sulfobutyl, 2-hydroxy-3- sulfopropyl, 2-(3-sulfopropoxy)-propyl, p-sulfobenzyl, and p-sulfophenethyl), a benzyl group, a phenethyl group, a vinylmethyl group, and the like,
X⁻ represents an acid anion (e.g. a chloride, bromide, iodide, thiocyanate, methylsulfate, ethylsulfate, perchlorate, and p-toluensulfonate ion), and
n represents 1 or 2.

The alkyl groups included in said substituents R₆, R₇, R₈, R₉, R₁₀, and R₁₁ and, more particularly, the alkyl portions of said alkoxy, alkoxycarbonyl, alkoxycarbonylamino, hydroxyalkyl, acetoxyalkyl groups and of the alkyl groups associated with a carboxy or sulfo group each preferably contain from 1 to 12, more preferably from 1 to 4 carbon atoms, the total number of carbon atoms included in said groups preferably being no more than 20.

The aryl groups included in said substituents R₆, R₇, R₈ and R₉ each preferably contain from 6 to 18, more preferably from 6 to 10 carbon atoms, the total number of carbon atoms included in said groups arriving up to 20 carbon atoms.

The following are specific examples of J-band sensitizing dyes belonging to those represented by the general formula (II) above:

According to the present invention, it has been found that the intensity of the sharp absorption band (J-band) shown by the spectral sensitizing dye adsorbed on the surface of the light-insensitive silver halide grains will vary with the quantity of the specific dye chosen as well as the size and chemical composition of the grains. The maximum intensity of J-band has been obtained with silver halide grains having the hereinbefore described sizes and the chemical compositions adsorbed with J-band spectral sensitizing dyes in a concentration of from 25 to 100 percent or more of monolayer coverage of the total available surface area of said silver halide grains. Optimum dye concentration levels can be chosen in the range of 0.5 to 20 millimoles per mole of silver bromoiodide, preferably in the range of 2 to 10 millimoles.

The J-band spectral sensitizing dyes are preferably added to the fine grain low iodide silver bromoiodide emulsions in the presence of a water soluble iodide or bromide salt. The J-band exhibited by said dyes adsorbed on said grains has been found to be increased by the presence of said salts. Said salts are more advantageously added to the silver halide emulsion before dye digestion, that is the pause following dye addition; said pause is preferably made at a temperature of 40 to 60°C for a time of about 50 to 150 minutes. Typical water soluble salts include alkali metal, alkali earth metal and ammonium iodide and bromide such as ammonium, potassium, lithium, sodium, cadmium and strontium iodides and bromides. The amount of said water soluble iodide and bromide salts is advantageously in a range of from 50 to 5,000 mg per mole of silver, and preferably from 100 to 1,000 mg per mole of silver.

The fine grain low iodide silver bromoiodide substantially light-insensitive emulsions of the present invention can be prepared by any of well-known procedures. Very fine grain emulsions known in the art as "Lippmann" emulsions are useful herein. According to a preferred procedure these emulsions can be formed by a double jet precipitation process wherein water soluble bromide and iodide salt are added concurrently with water soluble silver salt to a reaction vessel containing a dispersing medium.

The dispersing medium for said silver bromoiodide grains can be chosen among those conventionally employed in the silver halide emulsions. Preferred dispersion media include hydrophilic colloids, such as proteins, protein derivatives, cellulose derivatives (e.g. cellulose esters), gelatin (e.g. acid or alkali treated gelatin), gelatin derivatives (e.g. acetylated gelatin, phthalated gelatin and the like), polysaccarides (e.g. dextran), gum arabic, casein and the like. It is also common to employ said hydrophilic colloids in combination with synthetic polymeric binders and peptizers such as acrylamide and methacrylamide polymers, polymers of alkyl and sulfoalkyl acrylates and methacrylates, polyvinyl alcohol and its derivatives, polyvinyl lactams, polyamides, polyamines, polyvinyl acetates, and the like. At the end of grain precipitation, water soluble salts are removed from the emulsion with procedures known in the art, such as ultrafiltration. Such substantially light-insensitive silver bromiodide grains are not chemically sensitized nor substantially physically ripened.

According to another aspect, the present invention refers to a silver halide light-sensitive element to be associated with X-ray intensifying screens and used in radiography.

Said light-sensitive silver halide element for use in radiography with X-ray intensifying screens according to the present invention comprises a transparent support base having coated on at least one of its sides, preferably on both of its sides, a spectrally sensitized silver halide emulsion layer and, between the support base and the silver halide emulsion layer, a hydrophilic colloid layer containing substantially light-insensitive silver halide grains on which a spectral sensitizing dye is adsorbed, said dye adsorbed on said grains having the absorption in a region of the electromagnetic spectrum corresponding substantially to the spectral sensitivity of the silver halide emulsion, wherein said substantially light-insensitive silver halide grains are low iodide silver bromoiodide grains having an average grain size in the range of from 0.01 to 0.1 µm adsorbed with said spectral sensitizing dye to form a J-band as hereinbefore described.

The light-sensitive element comprises a polymeric base of the type commonly used in radiography, for instance a polyester base, in particular a polyethylene terephthalate base.

On at least one surface, preferably on both surfaces of the base there is coated a silver halide emulsion layer in a hydrophilic colloid. The emulsions coated on the two surfaces may also be different and comprise emulsions commonly used in photographic elements, such as silver chloride, silver iodide, silver chloro-bromide, silver chloro-bromo-iodide, silver bromide and silver bromo-iodide emulsions, the silver bromo-iodide emulsions being particularly useful for the X-ray elements. The silver halide crystals may have different shapes, for instance cubic, octahedral, spherical, tabular shapes, and may have epitaxial growth; they generally have mean sizes ranging from 0.2 to 3 micron, more preferably from 0.4 to 1.5 micron. The emulsions are coated on the base at a total silver coverage comprised in the range from about 3 to 6 grams per square meter. The silver halide binding material used is a water-permeable hydrophilic colloid, which is preferably gelatin, but other hydrophilic colloids, such as gelatin derivatives, albumin, polyvinyl alcohol, alginates, cellulose hydrolized esters, hydrophilic polyvinyl polymers, dextrans, polyacrylamides, acrylamide hydrophilic copolymers and alkylacrylates can also be used alone or in combination with gelatin.

The light-sensitive element according to the present invention is associated with the intensifying screens so as to be exposed to the radiations emitted by said screens. The screens are made of relatively thick phosphor layers which transform the x-rays into light radiation (e. g., visible light). The screens absorb a portion of x-rays much larger than the light-sensitive element and are used to reduce the radiation doses necessary to obtain a useful image. According to their chemical composition, the phosphors can emit radiations in the blue, green or red region of the visible spectrum and the silver halide emulsions are sensitized to the wavelength region of the light emitted by the screens. Sensitization is performed by using spectral sensitizers as well-known in the art. The x-ray intensifying screens used in the practice of the present invention are phosphor screens well-known in the art. Particularly useful phosphors are the rare earth oxysulfides doped to control the wavelength of the emitted light and their own efficiency. Preferably are lanthanum, gadolinium and lutetium oxysulfides doped with trivalent terbium as described in US patent 3,725,704. Among these phosphors, the preferred ones are gadolinium oxysulfides wherein from about 0.005% to about 8% by weight of the gadolinium ions are substituted with trivalent terbium ions, which upon excitation by UV radiations, x-rays, cathodic rays emit in the blue-green region of the spectrum with a main emission line around 544 nm. The silver halide emulsions are spectrally sensitized to the spectral region of the light emitted by the screens, preferably to a spectral region of an interval comprised within 25 nm from the wavelength of maximum emission of the screen, more preferably within 15 nm, and most preferably within 10 nm. Many types and combinations of spectral sensitizers can be used. In a preferred form of the present invention particularly useful spectral sensitizing dyes are those which exhibit an absorption peak (J-band) in their aggregated state. In a preferred form of the present invention, particularly useful spectral sensitizing dyes are those represented by the general formula (I) above. In the most preferred form of the present invention, wherein the phosphors of the screens are the gadolinium oxysulfides doped with trivalent terbium ions which emit light radiation comprised in the blue-green region of the visible spectrum, particularly useful dyes are those represented by formula (II) above and specific examples of dyes which absorb in the spectral region of emission of the gadolinium oxysulfides doped with trivalent terbium ions are those reported hereinabove. Preferably, the spectral sensitizing dye adsorbed on the light-sensitive silver halide grains has the same formula of the spectral sensitizing dye adsorbed on the substantially light-insensitive very fine grain low iodide silver bromoiodide grains as hereinbefore described.

The hydrophilic colloid layer containing the substantially light-insensitive very fine grain low iodide silver bromoiodide emulsions is a layer coated between the base and the silver halide emulsion layer. It is apparent that in a radiographic element having both surfaces of the support coated with light-sensitive emulsion layers either of the light-insensitive layers according to the present invention employed alone can effectively reduce crossover from both screens. Thus, only one light-insensitive layer is required, although for manufacture convenience double coated radiographic elements most commonly employ identical light-insensitive layers on opposite surfaces of the support. The hydrophilic colloid may be any colloid of the type generally used in the photographic elements as said above for the emulsion layer, the preferred colloid being gelatin. The layer may be either an intermediate auxiliary layer coated between the subbing layer of the base and the emulsion layer or the same subbing layer of the base. As known, in fact, the photographic base is per se hydrophobic and needs a hydrophilic layer, viz. the subbing layer, to assure sufficient adhesion of the light-sensitive hydrophilic layers. The use of the subbing layer, which normally consists of gelatin, to contain the substantially light-insensitive very fine grain low iodide silver bromoiodide emulsions according to the subject invention has the advantage of eliminating one layer, thus allowing a lower thickness of the photographic material and shorter drying times during the photographic processing. The thickness of the layer containing the substantially light-insensitive very fine grain low iodide silver bromoiodide emulsions according to the present invention is the normal thickness of layers used in the photographic elements as non light-sensitive layers (such as intermediate auxiliary layers or sublayers). Generally, said thickness ranges from 0.05 to 2 micron. Within such a range, as known in the art, a lower thickness, e.g. between 0.05 to 0.5 micron, is used when the layer works as a sublayer and a higher thickness, e.g. between 1 and 2 micron, is used when the layer works as a intermediate auxiliary layer. Besides, as known to the skilled in the art, the coating techniques used to coat the sublayer, i.e. the air knife coating technique, allow thinner layers than the coating techniques used to coat the auxiliary layers, e.g. the extrusion coating technique.

The sharp absorption band (J-band) shown by the spectral sensitizing dye adsorbed on the light-insensitive silver bromoioide grains of the layer coated between the base and the light-sensitive silver halide emulsion layer according to the present invention has the aim of absorbing the light emitted by the intensifying screens and therefore of avoiding or reducing the cross-over phenomenon. Of course, the higher the optical absorbance of the light-insensitive layer measured at the wavelength corresponding to the main emission peak of the phosphors, the better the image quality of the material, but at the same time the lower the sensitivity. Therefore, the man skilled in the art can choose the J-band absorbance by properly selecting the type and amount of spectral sensitizing dye adsorbed on the light-insensitive silver bromoiodide grains, the amount of water soluble iodide and bromide salts as hereinbefore described as well as the silver coating coverage according to the desired ratio between image quality (crossover) and sensitivity. Particularly useful optical absorbances are in the range from 0.3 to 1.50 read at the wavelength corresponding to the spectral emission maximum of the screens. The cross-over reduction attained with the light-insensitive layer according to this invention is preferably at least 10%, more preferably at least 20% and most preferably at least 30% lower than the cross-over which can be obtained without said light-insensitive layer. Within such a range, lower values of absorbance provide X-ray elements having a high sensitivity and good image qualities. Higher values of absorbance provide X-ray materials having a good sensitivity and high image quality. The absorbance above does not consider the possible optical density of the base. As known to the man skilled in the art, this may contain a dye, usually an anthraquinone blue dye as described in US patents 3,488,195 and 3,948,664 and in GB patent 968,244, which can have an absorption in the spectral region of the light emitted by the screens. Since such a dye incorporated in the base which is impermeable to the photographic processing, cannot be decolorized, the quantity used and the absorbance resulting therefrom are very low, the latter being generally in the range from 0.03 to 0.20 .

In addition to the capacity of the silver bromoiodide grains described above to reduce crossover, said grains are advantageous in that they can be readily removed (i.e., fixed) in processing with the undeveloped silver halide grains of the light-sensitive silver halide emulsion layer, thus avoiding any residual stain of the image bearing radiographic element.

While the light-insensitive silver bromoiodide emulsions heretofore described may be employed alone for crossover reduction, it is recognized that they can be empolyed in combination with conventional approaches for crossover reduction, if desired. A variety of approaches have been suggested to reduce crossover, as illustrated by Research Disclosure, Vol. 184, August 1979, Item 18431, Section V, here incorporated by reference.

Preferably, radiographic elements according to this invention having highly desirable image characteristics are those which employ in the light-sensitive silver halide emulsion layer low aspect ratio cubic silver halide grains having J-band spectral sensitizing dyes adsorbed on the surface of said silver halide grains in an amount substantially higher than that amount which substantially optimally sensitizes said grains, as described in European Patent Application 244,718.

Said substantially higher amount means a quantity which is required to obtain, in a double side coated radiographic element, a reduction of the cross-over exposure of at least 5% from the cross-over effect exhibited without such additional amount of dye. In quantitative terms, it generally means about 1.5 times the quantity minimally necessary to optimally sensitize the emulsion.

Said light-sensitive silver halide emulsions comprise a dispersing medium and low aspect ratio cubic silver halide grains. The term "cubic grains" according to the present invention is intended to include substantially cubic grains, that is silver halide grains which are regular cubic grains bounded by crystallographic faces (100), or which may have rounded edges and/or vertices or small faces (111), or may even be nearly spherical when prepared in the presence of soluble iodides or strong ripening agents, such as ammonia. The aspect ratio, that is the ratio of diameter to thickness, of said cubic silver halide grains is lower than 8:1, preferably lower than 5:1 and most preferably is less than 3:1 and about 1:1. The silver halide grains may be of any required composition for forming a negative silver image, such as silver chloride, silver bromide, silver iodide, silver chloro-bromide, silver bromo-iodide and the like. Particularly good results are obtained with silver bromoiodide grains, preferably silver bromo-iodide grains containing about 0.1 to 15% moles of iodide ions, more preferably about 0.5 to 10% moles of iodide ions and still preferably silver bromo-iodide grains having average grain sizes in the range from 0.2 to 3µ, more preferably from 0.4 to 1.5 µ.

Said cubic grain silver halide emulsions can be prepared by conventional methods, such as described in Research Disclosure, Vol. 176, December 1978, Item 17643. According to one preferred procedure, these emulsions can be prepared by a double jet precipitation process. Into a conventional reaction vessel for silver halide precipitation, equipped with an efficient stirring mechanism, is introduced a dispersing medium. Typically the dispersion medium initially introduced into the reaction vessel is about 10 to 50% by weight, preferably is about 20% by weight, based on the total weight of the dispersion medium present in the silver halide emulsion at the end of grain precipitation, the remaining portion of the dispersion medium being added after having removed the water soluble salts at the completion of silver halide precipitation. During precipitation, silver and halide salts are added to the reaction vessel by techniques well known in the precipitation of silver halide grains. Typically, an aqueous solution of a soluble silver salt, such as silver nitrate, is introduced into the reaction vessel concurrently with the introduction of the halide salts. A high pH, preferably a pH of about 9 to 11, in the reaction vessel favours the formation of the cubic grains. Said pH may be maintained during all the precipitation process or during part of said process. Particularly good results are obtained by precipitating about 10 to 30% by weight of the silver halide grains at a low pH, preferably from about 5 to 6, and the remaining silver halide grains at said high pH.

The dispersing medium for the silver halide grains can be chosen among those conventionally employed in the silver halide emulsions. Preferred dispersion media include hydrophilic colloids, such as proteins, protein derivatives, cellulose derivatives (e.g. cellulose esters), gelatin (e.g. acid or alkali treated gelatin), gelatin derivatives (e.g. acetylated gelatin, phthalated gelatin and the like), polysaccarides (e.g. dextran), gum arabic, casein and the like. It is also common to employ said hydrophylic colloids in combination with synthetic polymeric binders and peptizers such as acrylamide and methacrylamide polymers, polymers of alkyl and sulfoalkyl acrylates and methacrylates, polyvinyl alcohol and its derivatives, polyvinyl lactams, polyamides, polyamines, polyvinyl acetates, and the like.

The cubic grain silver halide emulsions may be chemically sensitized by any procedure known in the photographic art. The emulsion may be digested with active gelatins or with sulfur-containing compounds such as sodium thiosulfate, allylthiocyanate, allylthiourea, and the like. The silver halide emulsions may be sensitized by means of reductors, e.g. tin compounds as described in GB 789,823, polyamines and small amounts of noble metal compounds, such as gold, platinum, iridium, ruthenium and rhodium.

The cubic grain silver halide emulsions of the radiographic elements of the present invention are spectrally sensitized. According to the present invention, said spectral sensitizing dyes are employed in an amount substantially higher than that necessary to substantially optimally sensitize the cubic silver halide grains, preferably in an amount from two to eight times said optimum amount, more preferably in an amount from three to five times said optimum amount. Preferred amounts of spectral sensitizers in the photographic emulsion are in the range from 0.5 to 2 millimoles per mole of silver halide. More preferred quantities range from 0.6 to 1.2 millimoles per mole of silver halide.

It is known in the photographic art that photographic speed obtainable from the silver halide grains increases with the increasing concentration of the sensitizing dye until maximum speed is obtained with an optimum dye concentration, after that, further increases in dye concentration cause a decrease in the obtainable speed. The optimum amount of dye employed can vary depending upon the specific dye, as well as upon the size and aspect of the grains. Surprisingly, the amount of dye adsorbed on the surface of the low aspect ratio cubic grain silver halide emulsions of the light-sensitive layer can be increased beyond the optimum dye concentration to obtain in combination with the substantially light-insensitive J-band forming silver bromoiodide grains of the light-insensitive layer the full advantages of this invention, i.e. a reduced light scattering and cross-over exposure without a significant loss in speed.

The J-band sensitization dyes are preferably added to the low aspect ratio cubic grain silver halide emulsions in the presence of a water soluble iodide or bromide salt. The J-band sensitization is increased by the presence of said salts, increasing the strong coloration of the element before processing and consequently reducing the cross-over of exposing radiations by adding a smaller amount of dye. The residual stain after processing of the radiographic element also is lower. Said salts are more advantageously added to the silver halide emulsion before dye digestion, that is the pause following dye addition; said pause is preferably made at a temperature of 40 to 60°C for a time of about 50 to 150 minutes.

Typical water soluble salts include alkali metal, alkali earth metal and ammonium iodide and bromide such as ammonium, potassium, lithium, sodium, cadmium and strontium iodides and bromides. The amount of said water soluble iodide and bromide salts is advantageously lower than 100 mg per mole of silver, and preferably ranges from about 40 to about 70 mg per mole of silver.

Other radiographic elements according to this invention having highly desirable imaging characteristics are those which employ one or more light-sensitive high aspect ratio tabular grain emulsions or intermediate aspect ratio tabular grain emulsions, as disclosed in US Patents 4,425,425 and 4,425,426. Preferred tabular grain emulsions for use in the radiographic elements of this invention are those in which tabular silver halide grains having a thickness of less than 0.5 µm, preferably less than 0.3 µm and optimally less than 0.2 µm, have an average aspect ratio of greater than 5:1, preferably greater than 8:1 and optimally greater than 12:1 and account for greater than 50 percent, preferably greater than 70 percent and optimally greater than 90 percent of the total projected area of the silver halide grains present in the emulsion. It is specifically contemplated to provide double coated radiographic elements according to this invention in which tabular grain emulsion layers are coated nearer the support than nontabular grain silver halide emulsion layers to reduce crossover, as illustrated in European Patent Application 84,637.

By employing light-sensitive low aspect ratio cubic grain silver halide or tabular grain silver halide emulsion layers as above described, which themselves reduce crossover, in combination with the light-insensitive low iodide silver bromoiodide emulsion layer according to this invention, radiographic elements exhibiting extremely low crossover levels can be achieved while also achieving high photographic speed and low residual stain.

The spectral sensitizing dyes can be used in the light-sensitive silver halide emulsion layers of the radiographic elements of this invention in combination among them or with other addenda, such as stabilizers, antifoggants, development modifiers, coating agents, brighteners and antistatic agents, which combination results in a supersensitization (that is, into a spectral sensitization higher than that which could be obtained with any dye or addendum used alone or would result from the additive effect of the dyes and addenda). Mechanisms and compounds responsible for supersensitization are described for example in Photographic Science and Engineering, 18, 418-430, (1974). In particular advantageous results are obtained according to this invention by combining the spectral sensitizing dyes with a supersensitizing amount of a polymeric compound having amino-allilydene-malononitrile moieties, as described in US Pat. No. 4,307,183, such as copolymers of a vinyl addition monomers and 3-diallyl-amino-allylidene-malononitrile monomer.

In addition to the features specifically described above, the photographic elements of this invention, in the light-sensitive silver halide emulsion layers or in other layers, can include additional addenda of conventional nature, such as stabilizers, antifoggants, brighteners, absorbing materials, hardeners, coating aids, plasticizers, lubricants, matting agents, antikinking agents, antistatic agents, and the like, as described in Research Disclosure, Item 17643, December 1978 and in Research Disclosure, Item 18431, August 1979.

Preferred radiographic elements are of the type described in BE Patent 757,815 and in US Patent 3,705,858, i.e. elements wherein at least one light-sensitive silver halide emulsion layer is coated on both surfaces of a transparent support, the total silver coverage per surface unit for both layers being lower than about 6 g/m², preferably than 5 g/m². Such supports are preferably polyester film supports, such as polyethylene terephthalate films. Generally said supports for use in medical radiography are blue tinted. Preferred dyes are anthraquinone dyes, such as those described in US Patents 3,488,195; 3,849,139; 3,918,976; 3,933,502; 3,948,664 and in UK Patents 1,250,983 and 1,372,668.

The exposed radiographic elements can be processed by any of the conventional processing techniques. Such processing techniques are illustrated for example in Research Disclosure, Item 17643, cited above. Roller transport processing is particularly preferred, as illustrated in US Patents 3,025,779; 3,515,556; 3,545,971 and 3,647,459 and in UK Patent 1,269,268. Hardening development can be undertaken, as illustrated in US Patent 3,232,761.

As regards the processes for the silver halide emulsion preparation and the use of particular ingredients in the emulsion and in the light-sensitive element, reference is made to Research Disclosure 18,431 published in August 1979, wherein the following chapters are dealt with in deeper details:
- IA.: Preparation, purification and concentration methods for silver halide emulsions.
- IB.: Emulsion types.
- IC.: Crystal chemical sensitization and doping.
- II.: Stabilizers, antifogging and antifolding agents.
- IIA.: Stabilizers and/or antifoggants.
- IIB.: Stabilization or emulsions chemically sensitized with gold compounds.
- IIC.: Stabilization of emulsions containing polyalkylene oxides or plasticizers.
- IID.: Fog caused by metal contaminants.
- IIE.: Stabilization of materials comprising agents to increase the covering power.
- IIF.: Antifoggants for dichroic fog.
- IIG.: Antifoggants for hardeners and developers comprising hardeners.
- IIH.: Additions to minimize desensitization due to folding.
- III.: Antifoggants for emulsions coated on polyester bases.
- IIJ.: Methods to stabilize emulsions at safety lights.
- IIK.: Methods to stabilize x-ray materials used for high temperature. Rapid Access, roller processor transport processing.
- III.: Compounds and antistatic layers.
- IV.: Protective layers.
- V.: Direct positive materials.
- VI.: Materials for processing at room light.
- VII.: X-ray color materials.
- VIII.: Phosphors and intensifying screens.
- IX.: Spectral sensitization.
- X.: UV-sensitive materials
- XII.: Bases

### EXAMPLE 1

A reaction vessel equipped with a stirrer was charged with 7 L of water containing 70 g of gelatin and 4.5 ml of N/10 KBr. At 35°C a solution of 137 g KBr, 3.9 g KI and 23.5 g gelatin in 1.2 L of water and a solution of 200 g AgNO₃ in 1.2 L of water were added in 20 minutes according to conventional double jet techniques to the reaction vessel. The emulsion was washed in the conventional procedure. The silver bromoiodide grains exhibited a mean diameter of 0.066 µm and comprised 2 percent mole of silver iodide. The emulsion was added with KI in an amount of 400 mg/mole of silver and dye A in an amount of 5 g/mole of silver, added with surfactants and hardeners and coated on both sides of a transparent blue tinted polyester support at 0.195 g/m² Ag per side (Film 1A).

Following the procedure described above a film (Film 1B) was prepared using a silver bromoiodide emulsion having a mean diameter of 0.16 µm and 2 percent mole of silver iodide, was prepared.

The following Table 1 reports the measure of J-band made with reference to the spectrophotometric curve of each film in the region of 400 to 700 nm by measuring the absorbance at 549 nm, which corresponds to the dye absorbance J-band peak.

The J-band measurements demonstrate the major intensity of J-band peak with the use of a finer bromoiodide emulsion.

### EXAMPLE 2

Following the procedure described in example 1, the following silver halide (bromide, iodide or bromoiodide) emulsions were prepared:

Each emulsion was added with dye A in an amount of 5 g/mole of silver, added with surfactants and hardeners and coated on one side of a transparent blue tinted polyester support at 0.4 g/m² Ag.

The following Table 2 reports the measure of J-band peak at 549 nm for each film.

The J-band measurements demonstrate the major intensity of J-band peak with silver bromoiodide grains.

### EXAMPLE 3

Following the procedure described in Example 2, several films were prepared similar to film 2D but using different amounts of dye A.

The following Table 3 reports the measure of J-band peak at 549 nm for each film.

The J-band measurements demonstrate the increase of the J-band peak intensity obtained by increasing the amount of spectral sensitizing dye.

### EXAMPLE 4

A light-sensitive cubic grain silver bromo-iodide gelatin emulsion (having 2.3% mole iodide) was prepared. Said emulsion comprised cubic grains having an average diameter of about 0.7 µm and an average aspect ratio of about 1:1. The emulsion was chemically sensitized with a sulfur compound and a gold compound, and spectrally sensitized with 0.150 g/mole of silver of the green spectral sensitizing dye B and 208 mg/mole of silver of an (acrylamide-allylidenemalononitrile) copolymer containing about 9% w/w of aminoallylidenemalononitrile moieties. The emulsion, added with stabilizing and antifogging agents, surface active agents and gelatin hardeners, was coated on both sides of a subbed polyethylene terephthalate support base (blue tinted with an anthraquinone dye and having an optical density in green light of 0.13). The emulsion was coated at 2.35 g/m² silver and 1.9 g/m² gelatin per side. Each emulsion layer was finally covered with a protective gelatin layer at a gelatin coverage of 1.1 g/m². (Film 4A).

A light-insensitive fine grain silver bromo-iodide gelatin emulsion (having 2% iodide mole) was prepared. Said emulsion comprised grains having an average diameter of 0.057 µm. The emulsion was added with 7.5 g/ mole of silver of the green spectral sensitizing dye A and 400 mg/mole of silver of potassium iodide. The emulsion was coated on both sides of the support base above at 0.1 g/m² silver and 1.25 g/m² gelatin per side. Both surfaces of the film thus obtained were coated with silver halide emulsion layers and protective layers as Film 4A above. (Film 4B).

The light-insensitive fine grain silver bromo-iodide gelatin emulsion of Film 4B above, added with 7.5 g/ mole of silver of the green spectral sensitizing dye A and 400 mg/mole of silver of potassium iodide, was coated on both sides of the support base above at 0.15 g/m² silver and 1.25 g/m² gelatin per side. Both surfaces of the film thus obtained were coated with silver halide emulsion layers and protective layers as Film 4A above. (Film 4C).

The light-insensitive fine grain silver bromo-iodide gelatin emulsion of Film 4B above, added with 7.5 g/ mole of silver of the green spectral sensitizing dye A and 400 mg/mole of silver of potassium iodide, was coated on both sides of the support base above at 0.2 g/m² silver and 1.25 g/m² gelatin per side. Both surfaces of the film thus obtained were coated with silver halide emulsion layers and protective layers as Film 4A above. (Film 4D).

Each film was interposed between two green emitting 3M Trimax™ T8 intensifying screens, then exposed through a laminated aluminium step wedge to X-rays of 300 mA and 80 kV for 0.15 seconds. After the exposure, the films were processed in a 3M Trimatic™ XP 507 roller transport processor. Processing consisted of 3M XAD/2 Developer for 24 seconds at 35°C, followed by fixing in 3M XAF/2 Fixer for 24 seconds at 30°C, washing in tap water for 22 seconds at 35°C and drying for 22 seconds at 35°C.

The sensitometric and image quality results are tabulated in the following table. Percent cross-over has been calculated by using the following equation:$\text{Percent Cross-over =} \frac{\text{1}}{\text{antilog (δlog E)}} \text{x 100}$
wherein δlog E is the difference in sensitivity between the two emulsion layers of the same film when exposed with a single screen (the lower the percent of cross-over, the better the image quality). The measure of J-band was made referring to the spectrophotometric curve of the unexposed film in the region of 400 to 700 nm by measuring the absorbance at 549 nm, which correspond to the dye asorbance J-band peak near to the main emission peak of the phosphor of the screen.

### EXAMPLE 5

A light-sensitive cubic grain silver bromo-iodide gelatin emulsion (having 2.3% mole iodide) was prepared. Said emulsion comprised cubic grains having an average diameter of about 0.7 µm and an average aspect ratio of about 1:1. The emulsion was chemically sensitized with a sulfur compound and a gold compound, and spectrally sensitized with 0.150 g/mole of silver of the green spectral sensitizing dye B and 208 mg/mole of silver of an (acrylamide-allylidenemalononitrile) copolymer containing about 9% w/w of aminoallylidenemalononitrile moieties. The emulsion, added with stabilizing and antifogging agents, surface active agents and gelatin hardeners, was coated on both sides of a subbed polyethylene terephthalate support base (blue tinted with an anthraquinone dye and having an optical density in green light of 0.13). The emulsion was coated at 2.23 g/m² silver and 1.9 g/m² gelatin per side. Each emulsion layer was finally covered with a protective gelatin layer at a gelatin coverage of 1.1 g/m². (Film 5A).

A light-insensitive fine grain silver bromo-iodide gelatin emulsion (having 2% mole iodide) was prepared. Said emulsion comprised grains having an average diameter of 0.16 µm. The emulsion was added with 5.0 g/ mole of silver of the green spectral sensitizing dye A and 400 mg/mole of silver of potassium iodide. The emulsion was coated on both sides of the support base above at 0.2 g/m² silver and 1.25 g/m² gelatin per side. Both surfaces of the film thus obtained were coated with silver halide emulsion layers and protective layers as Film 5A above. (Film 5B).

A light-insensitive very fine grain silver bromoiodide gelatin emulsion (having 2% mole iodide) was prepared. Said emulsion comprised grains having an average diameter of 0.066 µm. The emulsion was added with 5.0 g/mole of silver of the green spectral sensitizing dye A and 400 mg/mole of silver of potassium iodide. The emulsion was coated on both sides of the support base above at 0.2 g/m² silver and 1.25 g/m² gelatin per side. Both surfaces of the film thus obtained were coated with silver halide emulsion layers and protective layers as Film 5A above. (Film 5C).

A cubic grain silver bromo-iodide gelatin emulsion (having 2.3% mole iodide) was prepared. Said emulsion comprised cubic grains having an average diameter of about 0.7 µm and an average aspect ratio of about 1:1. The emulsion was chemically sensitized with a sulfur compound and a gold compound, and spectrally sensitized with 0.750 g/mole of silver of the green spectral sensitizing dye A, 60 mg/mole of silver of potassium iodide and 208 mg/mole of silver of a (acrylamide-allylaminoallylidene-malononitrile) copolymer containing about 9% w/w of aminoallylidenemalononoitrile moieties. The emulsion, added with stabilizing and antifogging agents, surface active agents and gelatin hardeners, was coated on both sides of the subbed polyethylene terephthalate support base (blue-colored with an anthraquinone dye and having an optical density in green light of 0.13). The emulsion was coated at 2.25 g/m² silver and 1.9 g/m² gelatin per side. Each emulsion layer was finally covered with a protective gelatin layer at a gelatin coverage of 1.1 g/m². (Film 5D).

A light-insensitive fine grain silver bromo-iodide gelatin emulsion (having 2% mole iodide) was prepared. Said emulsion comprised grains having an average diameter of 0.16 µm. The emulsion was added with 5.0 g/ mole of silver of the green spectral sensitizing dye A and 400 mg/mole of silver of potassium iodide. The emulsion was coated on both sides of the support base above at 0.2 g/m² silver and 1.25 g/m² gelatin per side. Both surfaces of the film thus obtained were coated with silver halide emulsion layers and protective layers as Film 5D above. (Film 5E).

A light-insensitive very fine grain silver bromoiodide gelatin emulsion (having 2% mole iodide) was prepared. Said emulsion comprised grains having an average diameter of 0.066 µm. The emulsion was added with 5.0 g/mole of silver of the green spectral sensitizing dye A and 400 mg/mole of silver of potassium iodide. The emulsion was coated on both sides of the support base above at 0.2 g/m² silver and 1.25 g/m² gelatin per side. Both surfaces of the film thus obtained were coated with silver halide emulsion layers and protective layers as Film 5D above. (Film 5F).

Each film was interposed between two green emitting 3M Trimax™ T8 intensifying screens, then exposed through a laminated aluminium step wedge to X-rays of 300 mA and 80 kV for 0.15 seconds. After the exposure, the films were processed in a 3M Trimatic™ XP 507 roller transport processor. Processing consisted of 3M XAD/2 Developer for 24 seconds at 35°C, followed by fixing in 3M XAF/2 Fixer for 24 seconds at 30°C, washing in tap water for 22 seconds at 35°C and drying for 22 seconds at 35°C.

The sensitometric and image quality results are tabulated in the following table. Percent cross-over has been calculated by using the following equation:$\text{Percent Cross-over =} \frac{\text{1}}{\text{antilog (δlog E)}} \text{x 100}$
wherein δlog E is the difference in sensitivity between the two emulsion layers of the same film when exposed with a single screen (the lower the percent of cross-over, the better the image quality). The measure of J-band was made referring to the spectrophotometric curve of the unexposed film in the region of 400 to 700 nm by measuring the absorbance at 549 nm, which correspond to the dye asorbance J-band peak near to the main emission peak of the phosphor of the screen.

## Claims

1. A light-sensitive silver halide element for use in radiography with X-ray intensifying screens comprising a transparent support base having coated on at least one of its sides a spectrally sensitized silver halide emulsion layer and, between the support base and the silver halide emulsion layer, a hydrophilic colloid layer containing substantially light-insensitive low iodide silver bromoiodide grains on which a spectral sensitizing dye is adsorbed to form a J-band, said dye adsorbed on said grains having the absorption in a region of the electromagnetic spectrum corresponding substantially to the spectral sensitivity of the silver halide emulsion, characterized by the fact that said substantially light-insensitive low iodide silver bromoiodide grains have from more than 0.2 mole percent to less than 10 mole percent iodide and an average grain size in the range of from 0.01 to 0.1 µm.

2. The light-sensitive element of claim 1, wherein said spectrally sensitized silver halide emulsion layer is coated on both sides of the transparent support base.

3. The light-sensitive element of claim 1, wherein said spectral sensitizing dye adsorbed on said substantially light-insensitive silver halide grains is a cyanine dye.

4. The light-sensitive element of claim 1, wherein said dye adsorbed on said substantially light-insensitive silver halide grains exhibits a J-band as a function of the adsorption having an absorbance of at least 0.30.

5. The light-sensitive element of claim 1, wherein said dye adsorbed on said substantially light-insensitive silver halide grains is represented by the following general formula (I): wherein
Z₁ and Z₂, the same or different, each represents the elements necessary to complete a cyclic nucleus derived from basic heterocyclic nitrogen compounds,
R₁ and R₂, the same or different, each represents an alkyl group, an aryl group, an alkenyl group, or an aralkyl group,
R₃ represents a hydrogen atom,
R₄ and R₅, the same or different, each represents a hydrogen atom or a lower alkyl group,
p and q are 0 or 1,
m is 0 or 1,
A is an anionic group,
B is a cationic group, and
k and l may be 0 or 1.

6. The light-sensitive element of claim 1, wherein said dye adsorbed on said substantially light-insensitive silver halide grains is represented by the following general formula (II): wherein R₁₀ represents a hydrogen atom or a lower alkyl group, R₆, R₇, R₈ and R₉ each represents a hydrogen atom, a halogen atom, a hydroxy group, an alkoxy group, an amino group, an acylamino group, an acyloxy group, an alkoxycarbonyl group, an alkyl group, an alkoxycarbonylamino group or an aryl group, or, together, R₆ and R₇ and, respectively, R₈ and R₉ can be the atoms necessary to complete a benzene ring, R₁₁ and R₁₂ each represents an alkyl group, a hydroxyalkyl group, an acetoxyalkyl group, an alkoxyalkyl group, a carboxyl group containing alkyl group, a sulfo group containing alkyl group, a benzyl group, a phenetyl group or a vinylmethyl group, X⁻ represents an acid anion and n represents 1 or 2.

7. The light-sensitive element of claim 1, wherein said substantially light-insensitive silver halide grains are used in an amount of from 0.05 to 0.5 g/m².

8. The light-sensitive element of claim 1, wherein said dye adsorbed on said substantially light-insensitive silver halide grains is used in an amount of from 25 to 100 percent of monolayer coverage of the surface of said substantially light-insensitive silver halide grains.

9. The light-sensitive element of claim 1, wherein said spectral sensitizing dye adsorbed on said substantially light-insensitive silver halide grains is added to said substantially light-insensitive silver halide grains in reactive association with a water soluble iodide or bromide salt.

10. The light-sensitive element of claim 1, wherein the silver halide emulsion layer is spectrally sensitized to the green light of the visible spectrum.

11. The light-sensitive element of claim 1, wherein the silver halide emulsion layer comprises low aspect ratio cubic silver halide grains and a spectral sensitizing dye adsorbed on the surface of said cubic silver halide grains exhibiting a J-band as a function of the adsorption having an absorbance of at least 0.5.

12. The light-sensitive element of claim 11, wherein said spectral sensitizing dye is adsorbed on the surface of said cubic silver halide grains in an amount substantially higher than amount which substantially optimally sensitizes said cubic grains.

13. The light-sensitive element of claim 11, wherein the silver halide is a silver bromo-iodide having an average grain size in the range from 0.2 to 1.5 µm.

14. The light-sensitive element of claim 11, wherein said J-band spectral sensitizing dye is a cyanine dye.

15. The light-sensitive element of claim 11, wherein said dye adsorbed on said silver halide grains is represented by the following general formula (I): wherein
Z₁ and Z₂, the same or different, each represents the elements necessary to complete a cyclic nucleus derived from basic heterocyclic nitrogen compounds,
R₁ and R₂, the same or different, each represents an alkyl group, an aryl group, an alkenyl group, or an aralkyl group,
R₃ represents a hydrogen atom,
R₄ and R₅, the same or different, each represents a hydrogen atom or a lower alkyl group,
p and q are 0 or 1,
m is 0 or 1,
A is an anionic group,
B is a cationic group, and
k and l may be 0 or 1.

16. The light-sensitive element of claim 11, wherein said dye adsorbed on said silver halide grains is represented by the following general formula (II): wherein R₁₀ represents a hydrogen atom or a lower alkyl group, R₆, R₇, R₈ and R₉ each represents a hydrogen atom, a halogen atom, a hydroxy group, an alkoxy group, an amino group, an acylamino group, an acyloxy group, an alkoxycarbonyl group, an alkyl group, an alkoxycarbonylamino group or an aryl group, or, together, R₆ and R₇ and, respectively, R₈ and R₉ can be the atoms necessary to complete a benzene ring, R₁₁ and R₁₂ each represents an alkyl group, a hydroxyalkyl group, an acetoxyalkyl group, an alkoxyalkyl group, a carboxyl group containing alkyl group, a sulfo group containing alkyl group, a benzyl group, a phenetyl group or a vinylmethyl group, X⁻ represents an acid anion and n represents 1 or 2.

17. The light-sensitive element of claim 11, wherein said spectral sensitizing dye is adsorbed on the surface of the cubic silver halide grains in an amount of two to eight times the amount sufficient to optimally sensitize said grains.

18. The light-sensitive element of claim 11, wherein said spectral sensitizing dye is added to the cubic silver halide grains in reactive association with a water soluble iodide or bromide salt.

19. The light-sensitive element of claim 11, wherein said spectral sensitizing dye is added to the cubic silver halide grains in reactive association with a super-sensitizer.

20. The light-sensitive element of claim 11, wherein said spectral sensitizing dye is added to the cubic silver halide grains in reactive association with a super-sensitizing amount of a polymeric compound having an amino-allylidene-malononitrile moiety.

21. The light-sensitive element of claim 1, wherein the silver halide emulsion layer comprises tabular silver halide grains having a thickness of less than 0.5 µm and an average aspect ratio of at least 5:1 accounting for at least 35 percent of the total projected area of said silver halide grains present in said silver halide emulsion layer and a spectral sensitizing dye adsorbed on the surface of said tabular silver halide grains.

22. The light-sensitive element of claim 21, wherein said spectral sensitizing dye adsorbed on the surface of said tabular silver halide grains exhibits a J-band as a function of the adsorption having an absorbance of at least 0.5.

23. The light-sensitive element of claim 22, wherein said J-band spectral sensitizing dye is a cyanine dye.

24. The light-sensitive element of claim 21, wherein said dye adsorbed on the surface of said tabular silver halide grains is represented by the following general formula (I): wherein
Z₁ and Z₂, the same or different, each represents the elements necessary to complete a cyclic nucleus derived from basic heterocyclic nitrogen compounds,
R₁ and R₂, the same or different, each represents an alkyl group, an aryl group, an alkenyl group, or an aralkyl group,
R₃ represents a hydrogen atom,
R₄ and R₅, the same or different, each represents a hydrogen atom or a lower alkyl group,
p and q are 0 or 1,
m is 0 or 1,
A is an anionic group,
B is a cationic group, and
k and l may be 0 or 1.

25. The light-sensitive element of claim 21, wherein said dye adsorbed on the surface of said tabular silver halide grains is represented by the following general formula (II): wherein R₁₀ represents a hydrogen atom or a lower alkyl group, R₆, R₇, R₈ and R₉ each represents a hydrogen atom, a halogen atom, a hydroxy group, an alkoxy group, an amino group, an acylamino group, an acyloxy group, an alkoxycarbonyl group, an alkyl group, an alkoxycarbonylamino group or an aryl group, or, together, R₆ and R₇ and, respectively, R₈ and R₉ can be the atoms necessary to complete a benzene ring, R₁₁ and R₁₂ each represents an alkyl group, a hydroxyalkyl group, an acetoxyalkyl group, an alkoxyalkyl group, a carboxyl group containing alkyl group, a sulfo group containing alkyl group, a benzyl group, a phenetyl group or a vinylmethyl group, X⁻ represents an acid anion and n represents 1 or 2.

26. The light-sensitive element of claim 21, wherein the dye adsorbed on the surface of said tabular silver halide grains is used in an amount of from 25 to 100 percent of monolayer coverage of the surface of said tabular silver halide grains.

27. The light-sensitive element of claim 21, wherein said silver halide is silver bromide or silver bromo-iodide.

28. A substantially light-insensitive silver halide emulsion comprising low iodide silver bromoiodide grains on which a spectral sensitizing dye is adsorbed to form a J-band, characterized by the fact that said low iodide silver bromoiodide grains have from more than 0.2 mole percent to less than 10 mole percent iodide and an average grain size of from 0.01 to 0.1 µm.

29. The substantially light-insensitive silver halide emulsion of claim 28, wherein said spectral sensitizing dye adsorbed on said substantially light-insensitive silver halide grains is a cyanine dye.

30. The substantially light-insensitive silver halide emulsion of claim 28, wherein said dye adsorbed on said substantially light-insensitive silver halide grains is represented by the following general formula (I): wherein
Z₁ and Z₂, the same or different, each represents the elements necessary to complete a cyclic nucleus derived from basic heterocyclic nitrogen compounds,
R₁ and R₂, the same or different, each represents an alkyl group, an aryl group, an alkenyl group, or an aralkyl group,
R₃ represents a hydrogen atom,
R₄ and R₅, the same or different, each represents a hydrogen atom or a lower alkyl group,
p and q are 0 or 1,
m is 0 or 1,
A is an anionic group,
B is a cationic group, and
k and l may be 0 or 1.

31. The substantially light-insensitive silver halide emulsion of claim 28, wherein said dye adsorbed on said substantially light-insensitive silver halide grains is represented by the following general formula (II): wherein R₁₀ represents a hydrogen atom or a lower alkyl group, R₆, R₇, R₈ and R₉ each represents a hydrogen atom, a halogen atom, a hydroxy group, an alkoxy group, an amino group, an acylamino group, an acyloxy group, an alkoxycarbonyl group, an alkyl group, an alkoxycarbonylamino group or an aryl group, or, together, R₆ and R₇ and, respectively, R₈ and R₉ can be the atoms necessary to complete a benzene ring, R₁₁ and R₁₂ each represents an alkyl group, a hydroxyalkyl group, an acetoxyalkyl group, an alkoxyalkyl group, a carboxyl group containing alkyl group, a sulfo group containing alkyl group, a benzyl group, a phenetyl group or a vinylmethyl group, X⁻ represents an acid anion and n represents 1 or 2.

32. The substantially light-insensitive silver halide emulsion of claim 28, wherein said dye adsorbed on said substantially light-insensitive silver halide grains is used in an amount of from 25 to 100 percent of monolayer coverage of the surface of said substantially light-insensitive silver halide grains.

33. The substantially light-insensitive silver halide emulsion of claim 28, wherein said spectral sensitizing dye adsorbed on said substantially light-insensitive silver halide grains is added to said substantially light-insensitive silver halide grains in reactive association with a water soluble iodide or bromide salt.

34. A process for forming an X-ray image which includes:
(a) exposing to X-rays through X-ray intensifying screens a spectrally sensitized silver halide element comprising coated on at least one side of a transparent support base at least a spectrally sensitized silver halide emulsion layer and, between the base and a silver halide emulsion layer, a hydrophilic colloid layer containing substantially light-insensitive low iodide bromoiodide grains on which a spectral sensitizing dye is adsorbed to form a J-band, said dye adsorbed on said grains having the absorption in a region of the electromagnetic spectrum corresponding substantially to the spectral sensitivity of the silver halide emulsion,
(b) developing,
(c) fixing with thiosulfate ions, and
(d) washing with water,
characterized by the fact that said low iodide silver bromoiodide grains have from more than 0.2 mole percent to less than 10 mole percent iodide and an average grain size in the range of from 0.01 to 0.1 µm adsorbed with said spectral sensitizing dye to form a J-band.

## Patentansprüche

1. Lichtempfindliches Silberhalogenidelement zur Verwendung in der Radiographie mit Röntgenstrahlen-Verstärkerschirmen, umfassend einen durchsichtigen Grundträger, der auf mindestens einer Seite eine Beschichtung mit einer spektral sensibilisierten Silberhalogenidemulsionsschicht und zwischen dem Grundträger und der Silberhalogenidemulsionsschicht eine hydrophile Kolloidschicht aufweist, die im wesentlichen lichtunempfindliche, einen niedrigen Iodidgehalt aufweisende Silberbromiodidkörner enthält, an die ein Spektral-Sensibilisierungsfarbstoff unter Bildung einer J-Bande adsorbiert ist, wobei der an den Körnern adsorbierte Farbstoff eine Absorption im Bereich des elektromagnetischen Spektrums aufweist, die im wesentlichen der Spektralempfindlichkeit der Silberhalogenidemulsion entspricht, gekennzeichnet durch die Tatsache, daß die im wesentlichen lichtunempfindlichen Silberbromiodidkörner mit einem niedrigen Iodgehalt mehr als 0,2 mol-% bis weniger als 10 mol-% Iodid und eine mittlere Korngröße im Bereich von 0,01 bis 0,1 µm aufweisen.

2. Lichtempfindliches Element nach Anspruch 1, in dem der durchsichtige Grundträger auf beiden Seiten mit der spektralsensibilisierten Silberhalogenidemulsionsschicht beschichtet ist.

3. Lichtempfindliches Element nach Anspruch 1, in dem der Spektral-Sensibilisierungsfarbstoff, der an den im wesentlichen lichtunempfindlichen Silberhalogenidkörnern adsorbiert ist, ein Cyaninfarbstoff ist.

4. Lichtempfindliches Element nach Anspruch 1, in dem der Farbstoff, der an den im wesentlichen lichtunempfindlichen Silberhalogenidkörnern adsorbiert ist, eine J-Bande als eine Funktion der Adsorption mit einer Extinktion von mindestens 0,30 zeigt.

5. Lichtempfindliches Element nach Anspruch 1, in dem der Farbstoff, der an den im wesentlichen lichtunempfindlichen Silberhalogenidkörnern adsorbiert ist, durch die folgende allgemeine Formel (I) dargestellt wird: in der Z₁ und Z₂ gleich oder verschieden sind und jeweils die Elemente darstellen, die zur Vervollständigung eines cyclischen Kernes notwendig sind, der sich von basischen heterocyclischen Stickstoffverbindungen ableitet,
R₁ und R₂ gleich oder verschieden sind und jeweils einen Alkylrest, einen Arylrest, einen Alkenylrest oder einen Aralkylrest darstellen,
R₃ ein Wasserstoffatom ist,
R₄ und R₅ gleich oder verschieden sind und jeweils ein Wasserstoffatom oder einen Niederalkylrest darstellen,
p und q 0 oder 1 sind,
m 0 oder 1 ist,
A ein anionischer Rest ist,
B ein kationischer Rest ist und
k und l 0 oder 1 sein können.

6. Lichtempfindliches Element nach Anspruch 1, in dem der Farbstoff, der an den im wesentlichen lichtunempfindlichen Silberhalogenidkörnern adsorbiert ist, durch die folgende allgemeine Formel (II) dargestellt wird: in der R₁₀ ein Wasserstoffatom oder einen Niederalkylrest darstellt,
R₆, R₇, R₈ und R₉ jeweils ein Wasserstoffatom, ein Halogenatom, einen Hydroxyrest, einen Alkoxyrest, einen Aminorest, einen Acylaminorest, einen Acyloxyrest, einen Alkoxycarbonylrest, einen Alkylrest, einen Alkoxycarbonylaminorest oder einen Arylrest darstellen, oder R₆ und R₇, bzw. R₈ und R₉, zusammen die zur Vervollständigung eines Benzolringes notwendigen Atome sein können,
R₁₁ und R₁₂ jeweils einen Alkylrest, einen Hydroxyalkylrest, einen Acetoxyalkylrest, einen Alkoxyalkylrest, einen Carboxylrest enthaltenden Alkylrest, einen Sulforest enthaltenden Alkylrest, einen Benzylrest, einen Phenethylrest oder einen Vinylmethylrest darstellen,
X⁻ ein Säureanion darstellt und
n 1 oder 2 ist.

7. Lichtempfindliches Element nach Anspruch 1, in dem die im wesentlichen lichtunempfindlichen Silberhalogenidkörner in einer Menge von 0,05 bis 0,5 g/m² verwendet werden.

8. Lichtempfindliches Element nach Anspruch 1, in dem der Farbstoff, der an den im wesentlichen lichtunempfindlichen Silberhalogenidkörnern adsorbiert ist, in einer Menge von 25 bis 100% der Monoschichtbeschichtung der Oberfläche der im wesentlichen lichtunempfindlichen Silberhalogenidkörner verwendet wird.

9. Lichtempfindliches Element nach Anspruch 1, in dem der Spektral-Sensibilisierungsfarbstoff, der an den im wesentlichen lichtunempfindlichen Silberhalogenidkörnern adsorbiert ist, zu den im wesentlichen lichtunempfindlichen Silberhalogenidkörnern in reaktiver Assoziierung mit einem wasserlöslichen Iodid- oder Bromidsalz gegeben wird.

10. Lichtempfindliches Element nach Anspruch 1, in dem die Silberhalogenidemulsionsschicht in bezug auf das grüne Licht des sichtbaren Spektrums spektral sensibilisiert wird.

11. Lichtempfindliches Element nach Anspruch 1, in dem die Silberhalogenidemulsionsschicht kubische Silberhalogenidkörner mit einem niedrigen Seitenverhältnis und einen Spektral-Sensibilisierungsfarbstoff umfaßt, der an der Oberfläche der kubischen Silberhalogenidkörner adsorbiert ist, die eine J-Bande als eine Funktion der Adsorption mit einer Extinktion von mindestens 0,5 aufweisen.

12. Lichtempfindliches Element nach Anspruch 11, in dem der Spektral-Sensibilisierungsfarbstoff an der Oberfläche der kubischen Silberhalogenidkörner in einer Menge adsorbiert ist, die im wesentlichen höher als die Menge ist, die im wesentlichen die kubischen Körner optimal sensibilisiert.

13. Lichtempfindliches Element nach Anspruch 11, in dem das Silberhalogenid ein Silberbromiodid mit einer mittleren Korngröße im Bereich von 0,2 bis 1,5 µm ist.

14. Lichtempfindliches Element nach Anspruch 11, in dem der J-Bande-Specktral-Sensibilisierungsfarbstoff ein Cyaninfarbstoff ist.

15. Lichtempfindliches Element nach Anspruch 11, in dem der an den Silberhalogenidkörnern adsorbierte Farbstoff durch die folgende allgemeine Formel (I) dargestellt wird: in der Z₁ und Z₂ gleich oder verschieden sind und jeweils die Elemente darstellen, die zur Vervollständigung eines cyclischen Kernes notwendig sind, der sich von basischen heterocyclischen Stickstoffverbindungen ableitet,
R₁ und R₂ gleich oder verschieden sind und jeweils einen Alkylrest, einen Arylrest, einen Alkenylrest oder einen Aralkylrest darstellen,
R₃ ein Wasserstoffatom ist,
R₄ und R₅ gleich oder verschieden sind und jeweils ein Wasserstoffatom oder einen Niederalkylrest darstellen,
p und q 0 oder 1 sind,
m 0 oder 1 ist,
A ein anionischer Rest ist,
B ein kationischer Rest ist und
k und l 0 oder 1 sein können.

16. Lichtempfindliches Element nach Anspruch 11, in dem der Farbstoff, der an den Silberhalogenidkörnern adsorbiert ist, durch die folgende allgemeine Formel (II) dargestellt wird: in der R₁₀ ein Wasserstoffatom oder einen Niederalkylrest darstellt,
R₆, R₇, R₈ und R₉ jeweils ein Wasserstoffatom, ein Halogenatom, einen Hydroxyrest, einen Alkoxyrest, einen Aminorest, einen Acylaminorest, einen Acyloxyrest, einen Alkoxycarbonylrest, einen Alkylrest, einen Alkoxycarbonylaminorest oder einen Arylrest darstellen, oder R₆ und R₇, bzw. R₈ und R₉, zusammen die zur Vervollständigung eines Benzolringes notwendigen Atome sein können,
R₁₁ und R₁₂ jeweils einen Alkylrest, einen Hydroxyalkylrest, einen Acetoxyalkylrest, einen Alkoxyalkylrest, einen Carboxylrest enthaltenden Alkylrest, einen Sulforest enthaltenden Alkylrest, einen Benzylrest, einen Phenethylrest oder einen Vinylmethylrest darstellen,
X⁻ ein Säureanion darstellt und
n 1 oder 2 ist.

17. Lichtempfindliches Element nach Anspruch 11, in dem der Spektral-Sensibilisierungsfarbstoff an der Oberfläche der kubischen Silberhalogenidkörner in einer Menge des 2 bis 8fachen der Menge adsorbiert ist, die ausreicht, um die Körner optimal zu sensibilisieren.

18. Lichtempfindliches Element nach Anspruch 11, in dem der Spektral-Sensibilisierungsfarbstoff zu den kubischen Silberhalogenidkörnern in reaktiver Assoziierung mit einem wasserlöslichen Iodid- oder Bromidsalz gegeben wird.

19. Lichtempfindliches Element nach Anspruch 11, in dem der Spektral-Sensibilisierungsfarbstoff zu den kubischen Silber halogenidkörnern in reaktiver Assoziierung zu einem Übersensibilisator gegeben wird.

20. Lichtempfindliches Element nach Anspruch 11, in dem der Spektral-Sensibilisierungsarbstoff zu den kubischen Silberhalogenidkörnern in reaktiver Assoziierung mit einer übersensibilisierenden Menge einer polymeren Verbindung gegeben wird, die eine Aminoallylidenmalonsäuredinitrilgruppe aufweist.

21. Lichtempfindliches Element nach Anspruch 1, in dem die Silberhalogenidemulsionsschicht tafelförmige Silberhalogenidkörner mit einer Dicke von weniger als 0,5 µm und einem mittleren Seitenverhältnis von mindestens 5:1, die mindestens 35% der gesamten vortretenden Fläche der in der Silberhalogenidemulsionsschicht vorhandenen Silberhalogenidkörner beanspruchen, und einen an der Oberfläche der tafelförmigen Silberhalogenidkörner adsorbierten SpektralSensibilisierungsfarbstoff umfaßt.

22. Lichtempfindliches Element nach Anspruch 21, in dem der Spektral-Sensibilisierungsfarbstoff, der an der Oberfläche der tafelförmigen Silberhalogenidkörner adsorbiert ist, eine J-Bande als Funktion der Adsorption mit einer Extinktion von mindestens 0,5 zeigt.

23. Lichtempfindliches Element nach Anspruch 22, in dem der J-Bande-Spektral-Sensibilisierungsfarbstoff ein Cyaninfarbstoff ist.

24. Lichtempfindliches Element nach Anspruch 21, in dem der Farbstoff, der an der Oberfläche der tafelförmigen Silberhalogenidörner adsorbiert ist, durch die folgende allgemeine Formel (I) dargestellt wird: in der Z₁ und Z₂ gleich oder verschieden sind und jeweils die Elemente darstellen, die zur Vervollständigung eines cyclischen Kernes notwendig sind, der sich von basischen heterocyclischen Stickstoffverbindungen ableitet,
R₁ und R₂ gleich oder verschieden sind und jeweils einen Alkylrest, einen Arylrest, einen Alkenylrest oder einen Aralkylrest darstellen,
R₃ ein Wasserstoffatom ist,
R₄ und R₅ gleich oder verschieden sind und jeweils ein Wasserstoffatom oder einen Niederalkylrest darstellen,
p und q 0 oder 1 sind,
m 0 oder 1 ist,
A ein anionischer Rest ist,
B ein kationischer Rest ist und
k und l 0 oder 1 sein können.

25. Lichtempfindliches Element nach Anspruch 21, in dem der Farbstoff, der an der Oberfläche der tafelförmigen Silberhalogenidkörner adsorbiert ist, durch die folgende allgemeine Formel (II) dargestellt wird: in der R₁₀ ein Wasserstoffatom oder einen Niederalkylrest darstellt,
R₆, R₇, R₈ und R₉ jeweils ein Wasserstoffatom, ein Halogenatom, einen Hydroxyrest, einen Alkoxyrest, einen Aminorest, einen Acylaminorest, einen Acyloxyrest, einen Alkoxycarbonylrest, einen Alkylrest, einen Alkoxycarbonylaminorest oder einen Arylrest darstellen, oder R₆ und R₇, bzw. R₈ und R₉, zusammen die zur Vervollständigung eines Benzolringes notwendigen Atome sein können,
R₁₁ und R₁₂ jeweils einen Alkylrest, einen Hydroxyalkylrest, einen Acetoxyalkylrest, einen Alkoxyalkylrest, einen Carboxylrest enthaltenden Alkylrest, einen Sulforest enthaltenden Alkylrest, einen Benzylrest, einen Phenethylrest oder einen Vinylmethylrest darstellen,
X⁻ ein Säureanion darstellt und
n 1 oder 2 ist.

26. Lichtempfindliches Element nach Anspruch 21, in dem der Farbstoff, der an der Oberfläche der tafelförmigen Silberhalogenidkörner adsorbiert ist, in einer Menge von 25 bis 100% der Monoschichtbeschichtung der Oberfläche der tafelförmigen Silberhalogenidkörner verwendet wird.

27. Lichtempfindliches Element nach Anspruch 21, in dem das Silberhalogenid Silberbromid oder Silberbromiodid ist.

28. Im wesentlichen lichtunempfindliche Silberhalogenidemulsion, die Silberbromiodidkörner mit einem niedrigen Iodidgehalt umfaßt, an die ein Spektral-Sensibilisierungsfarbstoff unter Bildung einer J-Bande adsorbiert ist, gekennzeichnet durch die Tatsache, daß die Silberbromiodidkörner mit einem niedrigen Iodgehalt Iodid in mehr als 0,2 mol-% bis weniger als 10 mol-% und mit einer mittleren Korngröße von 0,01 bis 0,1 µm aufweisen.

29. Im wesentlichen lichtunempfindliche Silberhalogenidemul sion nach Anspruch 28, in der der Spektral-Sensibilisierungsfarbstoff, der an den im wesentlichen lichtunempfindlichen Silberhalogenidkörnern adsorbiert ist, ein Cyaninfarbstoff ist.

30. Im wesentlichen lichtunempfindliche Silberhalogenidemulsion nach Anspruch 28, in der der Farbstoff, der an den im wesentlichen lichtunempfindlichen Silberhalogenidkörnern adsorbiert ist, durch die folgende allgemeine Formel (I) dargestellt wird: in der Z₁ und Z₂ gleich oder verschieden sind und jeweils die Elemente darstellen, die zur Vervollständigung eines cyclischen Kernes notwendig sind, der sich von basischen heterocyclischen Stickstoffverbindungen ableitet,
R₁ und R₂ gleich oder verschieden sind und jeweils einen Alkylrest, einen Arylrest, einen Alkenylrest oder einen Aralkylrest darstellen,
R₃ ein Wasserstoffatom ist,
R₄ und R₅ gleich oder verschieden sind und jeweils ein Wasserstoffatom oder einen Niederalkylrest darstellen,
p und q 0 oder 1 sind,
m 0 oder 1 ist,
A ein anionischer Rest ist,
B ein kationischer Rest ist und
k und l 0 oder 1 sein können.

31. Im wesentlichen lichtunempfindliche Silberhalogenidemulsion nach Anspruch 28, in der der Farbstoff, der an den im wesentlichen lichtunempfindlichen Silberhalogenidkörnern adsorbiert ist, durch die folgende allgemeine Formel (II) dargestellt wird: in der R₁₀ ein Wasserstoffatom oder einen Niederalkylrest darstellt,
R₆, R₇, R₈ und R₉ jeweils ein Wasserstoffatom, ein Halogenatom, einen Hydroxyrest, einen Alkoxyrest, einen Aminorest, einen Acylaminorest, einen Acyloxyrest, einen Alkoxycarbonylrest, einen Alkylrest, einen Alkoxycarbonylamino rest oder einen Arylrest darstellen, oder R₆ und R₇, bzw. R₈ und R₉, zusammen die zur Vervollständigung eines Benzolringes notwendigen Atome sein können,
R₁₁ und R₁₂ jeweils einen Alkylrest, einen Hydroxyalkylrest, einen Acetoxyalkylrest, einen Alkoxyalkylrest, einen Carboxylrest enthaltenden Alkylrest, einen Sulforest enthaltenden Alkylrest, einen Benzylrest, einen Phenethylrest oder einen Vinylmethylrest darstellen,
X⁻ ein Säureanion darstellt und
n 1 oder 2 ist.

32. Im wesentlichen lichtunempfindliche Silberhalogenidemulsion nach Anspruch 28, in der der Farbstoff, der an den im wesentlichen lichtunempfindlichen Silberhalogenidkörnern adsorbiert ist, in einer Menge von 25 bis 100% der Monoschichtbeschichtung der Oberfläche der im wesentlichen lichtunempfindlichen Silberhalogenidkörner verwendet wird.

33. Im wesentlichen lichtunempfindliche Silberhalogenidemulsion nach Anspruch 28, in der der Spektral-Sensibilisierungsfarbstoff, der an den im wesentlichen lichtunempfindlichen Silberhalogenidkörnern adsorbiert ist, zu den im wesentlichen lichtunempfindlichen Silberhalogenidkörnern in reaktiver Assoziierung mit einem wasserlöslichen Iodid- oder Bromidsalz gegeben wird.

34. Verfahren zur Herstellung eines Röntgenstrahlenbildes, das einschließt:
a) Belichten eines spektral sensibilisierten Silberhalogenidelementes durch Röntgenstrahlen-Verstärkerschirme mit Röntgenstrahlen, das eine Beschichtung von mindestens einer Seite eines durchsichtigen Grundträgers mit mindestens einer spektral sensibilisierten Silberhalogenidemulsionsschicht und zwischen dem Grundträger und der Silberhalogenidemulsionsschicht eine hydrophile Kolloidschicht umfaßt, die im wesentlichen lichtunempfindliche Silberbromiodidkörner mit einem niedrigen Iodidgehalt enthält, an die ein Spektral-Sensibilisierungsfarbstoff unter Bildung einer J-Bande adsorbiert ist, wobei der an den Körnern adsorbierte Farbstoff eine Absorption im Bereich des elektromagnetischen Spektrums aufweist, die im wesentlichen der Spektralempfindlichkeit der Silberhalogenidemulsion entspricht,
b) Entwickeln,
c) Fixieren mit Thiosulfationen und
d) Waschen mit Wasser,
gekennzeichnet durch die Tatsache, daß die lichtunempfindlichen Silberbromiodidkörener mit einem niedrigen Iodgehalt, an die der Sensibilisierungsfarbstoff unter Bildung einer J-Bande adsorbiert ist, mehr als 0,2 mol-% bis weniger als 10 mol-% Iodid und eine mittlere Korngröße im Bereich von 0,01 bis 0,1 µm aufweisen.

## Revendications

1. Elément photosensible à l'halogénure d'argent, destiné à être utilisé en radiographie avec des écrans renforçateurs de rayons X, comprenant un support transparent sur lequel sont appliquées, au moins sur l'un de ses côtés, une couche d'émulsion à l'halogénure d'argent à sensibilisation spectrale, et, entre le support et la couche d'émulsion à l'halogénure d'argent, une couche de colloïde hydrophile contenant des grains de bromo-iodure d'argent, à faible teneur en iodure, essentiellement insensibles à la lumière, grains par lesquels un colorant assurant la sensibilité spectrale est adsorbé pour former une bande J, ce colorant adsorbé par ces grains présentant une absorption dans une région du spectre électromagnétique correspondant essentiellement à la sensibilité spectrale de l'émulsion à l'halogénure d'argent, caractérisé en ce que les grains de bromo-iodure d'argent, à faible teneur en iodure, essentiellement insensibles à la lumière, contiennent plus de 0,2 % en moles et moins de 10 % en moles d'iodure, et ont une granulométrie moyenne comprise entre 0,01 et 0,1 µm.

2. Elément photosensible selon la revendication 1, dans lequel la couche d'émulsion à l'halogénure d'argent à sensibilisation spectrale est appliquée sur les deux côtés du support transparent.

3. Elément photosensible selon la revendication 1, dans lequel le colorant à sensibilisation spectrale, adsorbé par les grains d'halogénure d'argent essentiellement insensibles à la lumière, est un colorant de cyanine.

4. Elément photosensible selon la revendication 1, dans lequel le colorant adsorbé par les grains d'halogénure d'argent essentiellement insensibles à la lumière présente une bande J dont l'absorbance, en fonction de l'adsorption, est d'au moins 0,30.

5. Elément photosensible selon la revendication 1, dans lequel le colorant adsorbé par les grains d'halogénure d'argent essentiellement insensibles à la lumière est représenté par la formule générale (I) ci-après : dans laquelle
Z₁ et Z₂, qui sont identiques ou différents, représentent chacun les éléments nécessaires pour compléter un noyau cyclique dérivé de composés azotés hétérocycliques basiques,
R¹ et R₂, qui sont identiques ou différents, représentent chacun un groupe alkyle, un groupe aryle, un groupe alcényle ou un groupe aralkyle,
R₃ est un atome d'hydrogène,
R₄ et R₅, qui sont identiques ou différents, sont chacun un atome d'hydrogène ou un groupe alkyle inférieur,
p et q valent 0 ou 1,
m vaut 0 ou 1,
A est un groupe anionique,
B est un groupe cationique, et
k et l peuvent valoir 0 ou 1.

6. Elément photosensible selon la revendication 1, dans lequel le colorant adsorbé par les grains d'halogénure d'argent essentiellement insensibles à la lumière est représenté par la formule générale (II) ci-après : dans laquelle R₁₀ est un atome d'hydrogène ou un groupe alkyle inférieur, chacun des radicaux R₆, R₇, R₈ et R₉ est un atome d'hydrogène, un atome d'halogène, un groupe hydroxy, un groupe alcoxy, un groupe amino, un groupe acylamino, un groupe acyloxy, un groupe alcoxycarbonyle, un groupe alkyle, un groupe alcoxycarbonylamino ou un groupe aryle, ou encore R₆ et R₇ ou encore R₈ et R₉, pris ensemble, peuvent représenter les atomes nécessaires pour compléter un noyau benzénique, chacun des radicaux R₁₁ et R₁₂ est un groupe alkyle, un groupe hydroxyalkyle, un groupe acétoxyalkyle, un groupe alcoxyalkyle, un groupe alkyle contenant un groupe carboxyle, un groupe alkyle contenant un groupe sulfo, un groupe benzyle, un groupe phénéthyle ou un groupe vinylméthyle, X⁻ est un anion acide et n vaut 1 ou 2.

7. Elément photosensible selon la revendication 1, dans lequel les grains d'halogénure d'argent essentiellement insensibles à la lumière sont utilisés en une quantité de 0,05 à 0,5 g/m².

8. Elément photosensible selon la revendication 1, dans lequel le colorant adsorbé par les grains d'halogénure d'argent essentiellement insensibles à la lumière est utilisé en une quantité de 25 à 100 % de la monocouche couvrant la surface des grains d'halogénure d'argent essentiellement insensibles à la lumière.

9. Elément photosensible selon la revendication 1, dans lequel le colorant à sensibilisation spectrale, adsorbé par les grains d'halogénure d'argent essentiellement insensibles à la lumière, est ajouté aux grains d'halogénure d'argent essentiellement insensibles à la lumière dans le cadre d'une association de type réaction avec un iodure ou un bromure soluble dans l'eau.

10. Elément photosensible selon la revendication 1, dans lequel la couche d'émulsion à l'halogénure d'argent a subi une sensibilisation spectrale à la lumière verte du spectre visible.

11. Elément photosensible selon la revendication 1, dans lequel la couche d'émulsion à l'halogénure d'argent comprend des grains d'halogénure d'argent cubiques, à faible rapport d'aspect, et un colorant à sensibilisation spectrale adsorbé par la surface de ces grains d'halogénure d'argent cubiques présentant une bande J ayant, en fonction de l'adsorption, une absorbance d'au moins 0,5.

12. Elément photosensible selon la revendication 11, dans lequel le colorant à sensibilisation spectrale est adsorbé par la surface des grains d'halogénure d'argent cubiques en une quantité essentiellement supérieure à la quantité qui sensibilise d'une manière essentiellement optimale les grains cubiques.

13. Elément photosensible selon la revendication 11, dans lequel l'halogénure d'argent est un bromo-iodure d'argent ayant une granulométrie moyenne comprise entre 0,2 et 1,5 µm.

14. Elément photosensible selon la revendication 11, dans lequel le colorant à sensibilisation spectrale à bande J est un colorant de cyanine.

15. Elément photosensible selon la revendication 11, dans lequel le colorant adsorbé par les grains d'halogénure d'argent est représenté par la formule générale (I) ci-après : dans laquelle
Z₁ et Z₂, qui sont identiques ou différents, représentent chacun les éléments nécessaires pour compléter un noyau cyclique dérivé de composés azotés hétérocycliques basiques,
R¹ et R₂, qui sont identiques ou différents, représentent chacun un groupe alkyle, un groupe aryle, un groupe alcényle ou un groupe aralkyle,
R₃ est un atome d'hydrogène,
R₄ et R₅, qui sont identiques ou différents, sont chacun un atome d'hydrogène ou un groupe alkyle inférieur,
p et q valent 0 ou 1,
m vaut 0 ou 1,
A est un groupe anionique,
B est un groupe cationique, et
k et l peuvent valoir 0 ou 1.

16. Elément photosensible selon la revendication 11, dans lequel le colorant adsorbé par les grains d'halogénure d'argent est représenté par la formule générale (II) ci-après : dans laquelle R₁₀ est un atome d'hydrogène ou un groupe alkyle inférieur, chacun des radicaux R₆, R₇, R₈ et R₉ est un atome d'hydrogène, un atome d'halogène, un groupe hydroxy, un groupe alcoxy, un groupe amino, un groupe acylamino, un groupe acyloxy, un groupe alcoxycarbonyle, un groupe alkyle, un groupe alcoxycarbonylamino ou un groupe aryle, ou encore R₆ et R₇ ou encore R₈ et R₉, pris ensemble, peuvent représenter les atomes nécessaires pour compléter un noyau benzénique, chacun des radicaux R₁₁ et R₁₂ est un groupe alkyle, un groupe hydroxyalkyle, un groupe acétoxyalkyle, un groupe alcoxyalkyle, un groupe alkyle contenant un groupe carboxyle, un groupe alkyle contenant un groupe sulfo, un groupe benzyle, un groupe phénéthyle ou un groupe vinylméthyle, X⁻ est un anion acide et n vaut 1 ou 2.

17. Elément photosensible selon la revendication 11, dans lequel le colorant à sensibilisation spectrale est adsorbé par la surface des grains d'halogénure d'argent cubiques en une quantité de deux à huit fois supérieure à la quantité suffisante pour sensibiliser ces grains d'une manière optimale.

18. Elément photosensible selon la revendication 11, dans lequel le colorant à sensibilisation spectrale est ajouté aux grains d'halogénure d'argent cubiques en association de réaction avec un iodure ou un bromure soluble dans l'eau.

19. Elément photosensible selon la revendication 11, dans lequel le colorant à sensibilisation spectrale est ajouté aux grains d'halogénure d'argent cubiques en association de réaction avec un super-sensibilisateur.

20. Elément photosensible selon la revendication 11, dans lequel le colorant à sensibilisation spectrale est ajouté aux grains d'halogénure d'argent cubiques en association de réaction avec une quantité à effet de super-sensibilisation d'un composé polymère ayant un fragment amino-allylidène-malononitrile.

21. Elément photosensible selon la revendication 1, dans lequel la couche d'émulsion à l'halogénure d'argent comprend des grains d'halogénure d'argent lamellaires ayant une épaisseur inférieure à 0,5 µm et un rapport d'aspect moyen d'au moins 5:1, comptant pour au moins 35 % de la totalité de l'aire projetée des grains d'halogénure d'argent présents dans la couche d'émulsion à l'halogénure d'argent, et un colorant à sensibilisation spectrale, adsorbé par la surface des grains d'halogénure d'argent lamellaires.

22. Elément photosensible selon la revendication 21, dans lequel le colorant à sensibilisation spectrale, adsorbé par la surface des grains d'halogénure d'argent lamellaires, a une bande J dont l'absorbance, en fonction de l'adsorption, est d'au moins 0,5.

23. Elément photosensible selon la revendication 22, dans lequel le colorant à sensibilisation spectrale à bande J est un colorant de cyanine.

24. Elément photosensible selon la revendication 22, dans lequel le colorant adsorbé par la surface des grains d'halogénure d'argent lamellaires est représenté par la formule générale (I) ci-après : dans laquelle
Z₁ et Z₂, qui sont identiques ou différents, représentent chacun les éléments nécessaires pour compléter un noyau cyclique dérivé de composés azotés hétérocycliques basiques,
R¹ et R₂, qui sont identiques ou différents, représentent chacun un groupe alkyle, un groupe aryle, un groupe alcényle ou un groupe aralkyle,
R₃ est un atome d'hydrogène,
R₄ et R₅, qui sont identiques ou différents, sont chacun un atome d'hydrogène ou un groupe alkyle inférieur,
p et q valent 0 ou 1,
m vaut 0 ou 1,
A est un groupe anionique,
B est un groupe cationique, et
k et l peuvent valoir 0 ou 1.

25. Elément photosensible selon la revendication 21, dans lequel le colorant adsorbé par la surface des grains d'halogénure d'argent lamellaires est représenté par la formule générale (II) ci-après : dans laquelle R₁₀ est un atome d'hydrogène ou un groupe alkyle inférieur, chacun des radicaux R₆, R₇, R₈ et R₉ est un atome d'hydrogène, un atome d'halogène, un groupe hydroxy, un groupe alcoxy, un groupe amino, un groupe acylamino, un groupe acyloxy, un groupe alcoxycarbonyle, un groupe alkyle, un groupe alcoxycarbonylamino ou un groupe aryle, ou encore R₆ et R₇ ou encore R₈ et R₉, pris ensemble, peuvent représenter les atomes nécessaires pour compléter un noyau benzénique, chacun des radicaux R₁₁ et R₁₂ est un groupe alkyle, un groupe hydroxyalkyle, un groupe acétoxyalkyle, un groupe alcoxyalkyle, un groupe alkyle contenant un groupe carboxyle, un groupe alkyle contenant un groupe sulfo, un groupe benzyle, un groupe phénéthyle ou un groupe vinylméthyle, X⁻ est un anion acide et n vaut 1 ou 2.

26. Elément photosensible selon la revendication 21, dans lequel le colorant adsorbé par la surface des grains d'halogénure d'argent lamellaires est utilisé en une quantité de 25 à 100 % de la monocouche recouvrant la surface des grains d'halogénure d'argent lamellaires.

27. Elément photosensible selon la revendication 21, dans lequel l'halogénure d'argent est le bromure d'argent ou le bromo-iodure d'argent.

28. Emulsion à l'halogénure d'argent, essentiellement insensible à la lumière, comprenant des grains de bromo-iodure d'argent à faible teneur en iodure, par lesquels un colorant à sensibilisation spectrale est adsorbé pour former une bande J, caractérisée en ce que les grains de bromo-iodure d'argent à faible teneur en iodure contiennent plus de 0,2 % en moles et moins de 10 % en moles d'iodure, et ont une granulométrie moyenne de 0,01 à 0,1 µm.

29. Emulsion à l'halogénure d'argent essentiellement insensible à la lumière selon la revendication 28, dans laquelle le colorant à sensibilisation spectrale, adsorbé par les grains d'halogénure d'argent essentiellement insensibles à la lumière, est un colorant de cyanine.

30. Emulsion à l'halogénure d'argent essentiellement insensible à la lumière selon la revendication 28, dans laquelle le colorant adsorbé par les grains d'halogénure d'argent essentiellement insensibles à la lumière est représenté par la formule générale (I) ci-après : dans laquelle
Z₁ et Z₂, qui sont identiques ou différents, représentent chacun les éléments nécessaires pour compléter un noyau cyclique dérivé de composés azotés hétérocycliques basiques,
R¹ et R₂, qui sont identiques ou différents, représentent chacun un groupe alkyle, un groupe aryle, un groupe alcényle ou un groupe aralkyle,
R₃ est un atome d'hydrogène,
R₄ et R₅, qui sont identiques ou différents, sont chacun un atome d'hydrogène ou un groupe alkyle inférieur,
p et q valent 0 ou 1,
m vaut 0 ou 1,
A est un groupe anionique,
B est un groupe cationique, et
k et l peuvent valoir 0 ou 1.

31. Emulsion à l'halogénure d'argent essentiellement insensible à la lumière selon la revendication 28, dans laquelle le colorant adsorbé par les grains d'halogénure d'argent essentiellement insensibles à la lumière est représenté par la formule générale (II) ci-après : dans laquelle R₁₀ est un atome d'hydrogène ou un groupe alkyle inférieur, chacun des radicaux R₆, R₇, R₈ et R₉ est un atome d'hydrogène, un atome d'halogène, un groupe hydroxy, un groupe alcoxy, un groupe amino, un groupe acylamino, un groupe acyloxy, un groupe alcoxycarbonyle, un groupe alkyle, un groupe alcoxycarbonylamino ou un groupe aryle, ou encore R₆ et R₇ ou encore R₈ et R₉, pris ensemble, peuvent représenter les atomes nécessaires pour compléter un noyau benzénique, chacun des radicaux R₁₁ et R₁₂ est un groupe alkyle, un groupe hydroxyalkyle, un groupe acétoxyalkyle, un groupe alcoxyalkyle, un groupe alkyle contenant un groupe carboxyle, un groupe alkyle contenant un groupe sulfo, un groupe benzyle, un groupe phénéthyle ou un groupe vinylméthyle, X⁻ est un anion acide et n vaut 1 ou 2.

32. Emulsion à l'halogénure d'argent essentiellement insensible à la lumière selon la revendication 28, dans laquelle le colorant adsorbé par les grains d'halogénure d'argent essentiellement insensibles à la lumière est utilisé en une quantité de 25 à 100 % de la monocouche recouvrant la surface des grains d'halogénure d'argent essentiellement insensibles à la lumière.

33. Emulsion à l'halogénure d'argent essentiellement insensible à la lumière selon la revendication 28, dans laquelle le colorant à sensibilisation spectrale adsorbé par les grains d'halogénure d'argent essentiellement insensibles à la lumière est ajouté aux grains d'halogénure d'argent essentiellement insensibles à la lumière en association de réaction avec un iodure ou un bromure soluble dans l'eau.

34. Procédé pour former une image radiographique, qui consiste :
(a) à exposer à des rayons X, par l'intermédiaire d'écrans renforçateurs de rayons X, un élément à l'halogénure d'argent ayant subi une sensibilisation spectrale, comprenant, appliquées sur au moins un côté d'un support transparent, au moins une couche d'émulsion à l'halogénure d'argent ayant subi une sensibilisation spectrale, et, entre le support et une couche d'émulsion à l'halogénure d'argent, une couche de colloïde hydrophile contenant des grains de bromo-iodure d'argent à faible teneur en iodure et essentiellement insensibles à la lumière, par lesquels un colorant à sensibilisation spectrale est adsorbé pour former une bande J, ce colorant adsorbé par les grains ayant une absorption dans une région du spectre électromagnétique correspondant essentiellement à la sensibilisation spectrale de l'émulsion à l'halogénure d'argent,
(b) à développer,
(c) à fixer avec des ions thiosulfate, et
(d) à laver à l'eau,
caractérisé en ce que les grains de bromo-iodure d'argent à faible teneur en iodure contiennent plus de 0,2 % en moles et moins de 10 % en moles d'iodure et ont une granulométrie moyenne comprise entre 0,01 et 0,1 µm, ayant adsorbé le colorant à sensibilisation spectrale pour former une bande J.
